

# UNITED STATES PATENT OFFICE.

AUGUSTE JEAN BAPTISTE TAULEIGNE, OF PONTIGNY, AND ELIE MAZO, OF PARIS,  
FRANCE.

## PROCESS OF PHOTOGRAPHY IN COLORS.

1,059,917.

Specification of Letters Patent. Patented Apr. 22, 1913.

No Drawing.

Application filed March 23, 1910. Serial No. 551,135.

*To all whom it may concern:*

Be it known that we, AUGUSTE JEAN BAPTISTE TAULEIGNE, of Pontigny, Yonne, Republic of France, priest, and ELIE MAZO, of 5 8 Boulevard de Magenta, in the city of Paris, Republic of France, manufacturer of photographic apparatus, have invented an Improved Process of Photography in Colors, of which the following is a full, clear, and 10 exact description.

The object of the present invention is to enable photographic positives to be obtained in all shades, by the transformation of an ordinary silver positive into an anilin monochrome.

The present improved process can be employed for; 1st, obtaining simple positives in all shades on glass or on paper; 2nd, obtaining superposed bi-colored double prints 20 for projection in relief; 3rd, obtaining trichrome positive for color photography.

Many of the principles on which the present process is based are already known.

The present invention comprises a complete series of operations, and the use of various reagents, which result in the production of perfect pictures.

It is known that certain bodies, in particular the metallic salts of various groups, 30 have the property of precipitating several anilin colors. Such salts include many of the chlorids, bromids, ferricyanids, and others. Among these, the most interesting for the purpose now in hand, are the chlorid, iodid, ferricyanid and chromate of silver, because it is easy to transform the reduced silver of photographs into any one of these compounds. The salt that has given the best results and which forms the object 40 of the present patent is iodid of silver obtained by double transformation: 1st. of reduced silver into chlorid, bromid or ferricyanid of silver; 2nd. by transformation of these compounds into iodid of silver by the 45 action of iodid of potassium.

The detail of the operations which this process comprises is the following: The positive after being well freed from hyposulfite is plunged in a solution of bichlorid

of copper. Soon after the image whitens 50 by being transformed into chlorid of silver or more probably into double chlorid of silver and of copper. If this first transformation was to be made into bromid of silver, the print would be immersed in a 55 bromid at the maximum concentration, such as ferric bromid, and if it was to be made into ferrocyanid, ferricyanid of potassium would be used. The concentration of these reagents is of small importance. When the 60 transformation is complete, the print is washed in order to free it from the reagent, then it is plunged in a very weak solution of iodid of potassium: 1% or 2% at the maximum. In this bath the color of the image 65 which was a brownish white is changed to a greenish white and the print is transformed into iodid of silver or more probably into double iodid of silver and of copper, or of silver and of iron, or of silver and of potassium according to the reagent used in the 70 first transformation. This double transformation is extremely important since by direct transformation the monochromes obtained are not sufficiently intense. After this transformation of the image, immersion in a dye-bath follows. A sufficient though small number of anilin colors react well in the presence of iodid of silver. Those which operate 75 the best are: the red of rosanilin or fuchsin, the blue of methylene, or the blue commonly known as blue 149, and ordinary auromin, for trichromes. For by-color prints intended for stereoscopic projection, a mixture of fuchsin and auromin in predetermined proportions, and the green known to commerce by the name of brilliant green or ethyl green, is preferred. The aqueous solutions of these 80 several coloring matters should be relatively weak and contain a small proportion of acetic acid, which favors imbibition while preventing the filling up of the whites. However the degree of concentration need not be rigorously insisted upon and a weak 85 bath, in course of time, produces monochromes as intense as those produced by a concentrated bath.

The image of iodid of silver on the print,

after being washed for some minutes in order to eliminate iodid of potassium, is plunged into the selected coloring solution. The time of imbibition is about 12 hours. 5 The termination of this operation can be noted by observing when the coloration is as intense on the back as on the face of the plate or film-carrier. If the whites are tinted, the print is cleared or washed out 10 either in plain water, or in water containing a small quantity of acetic acid. After this the most important operation takes place. In this last mentioned operation the silver salt of the sensitive film is caused to 15 vanish without removing the color and even without permitting it to diffuse through the gelatin. Two methods are available.

According to one method the print is fixed 20 in a bath of iodid of potassium of 20% strength. The iodid of silver is rendered completely transparent without however disappearing. The monochrome therefore has all the purity of color which characterizes the anilin color without fading or 25 fusing since iodid of silver is permanent.

The second method is much more general and more perfect. It is based on the two following operations. The monochrome is first plunged in a bath of tannin of from 30 3% to 10% concentration and left to rest for about 12 minutes. The tannin, which precipitates all anilin colors without exception, renders the color insoluble without affecting the iodid of silver, the fixing of the 35 print can therefore be thereafter accomplished without fear of injury.

Two methods of fixing are available after the treatment with tannin; the hyposulfite of soda method, and the cyanid of potassium method. For fixing by means of hyposulfite of soda, after having removed the greater part of the tannin contained in the sensitive film by a thorough washing, the print is plunged into a concentrated or saturated bath of hyposulfite. The period for fixing is about ten minutes. In a less concentrated bath the fixing will be difficult and often incomplete. It is now only necessary to eliminate the hyposulfite by a 45 thorough washing. The employment of tannin, besides being indispensable for fixing the colors, leaves them in the gelatin in a precipitated form which gives them an extraordinary solidity.

In order to fix by means of cyanid of potassium, the print, after the treatment with tannin, is plunged into a solution of cyanid of potassium of about 10% strength. The iodid of silver disappears very rapidly, 55 contrarily to what happens with the fixing by iodid of potassium which only renders the silver salt transparent without removing it, the fixing by hyposulfite and by cyanid determine a real dissolution and the 60 iodid of silver is completely eliminated.

The monochrome is then washed first in plain water in order to eliminate the excess of cyanid then in water slightly acidulated with acetic acid and finally washed with a large quantity of water.

Only prints with free tones formed solely by anilin colors have hereinabove been mentioned, but positives in less intense colors can be obtained. In this case, in place of fixing the positive after imbibition and washing out, the positive is passed through a bath of tannin, then washed, and the iodid of silver re-developed in any suitable developing bath. The print is, in this case, formed by reduced silver the tone or shade 80 of which is modified by the anilin color.

In conclusion, the present improved process for transforming a silver print into an anilin print, is quite a general process in which the order of the operations is as follows:—1. Transformation of reduced silver into chlorid of silver by bi-chlorid of copper. 2. Transformation of chlorid of silver into iodid of silver by a weak bath of iodid of potassium. 3. Imbibition in a weak bath 90 of a selected anilin color. 4. Washing the print in plain water or in acidulated water. 5. Fixing the color in a 3% to 10% solution of tannin. 6. Elimination of the excess tannin by means of plain water. 7. Elimination of the silver salt by means of concentrated hyposulfite of soda or by cyanid of potassium of about 10% strength. 8. Elimination of the fixing reagent by a final washing.

#### Claims—

1. The herein described steps in a process for the production of colored photographs from ordinary silver positives, which consists in the treatment of the positive with bi-chlorid of copper, subsequently treating it with iodid of potassium, immersing it in an anilin dye-bath, washing with water, fixing the color by immersion in a solution of tannin, washing to eliminate excess of tannin, fixing the print, and finally washing to eliminate the fixing reagent.

2. The herein described steps in a process for the production of colored photographs from ordinary silver positives, which consists in the treatment of the positive with bi-chlorid of copper, subsequently treating it with iodid of potassium, immersing it in an anilin dye-bath, washing with water, fixing the color by immersion in a 3% to 10% solution of tannin, washing to eliminate excess of tannin, fixing the print by means of hyposulfite of soda, and finally washing the print to eliminate the fixing reagent.

3. The herein described steps in a process for the production of colored photographs from ordinary silver positives, which consists in the treatment of the positive with bi-chlorid of copper, subsequently treating it with iodid of potassium, immersing it in 120

an anilin dye-bath, washing with water, fixing the color by immersion in a 3% to 10% solution of tannin, washing to eliminate excess of tannin, fixing the print by means of a concentrated solution of hyposulphite of soda, and finally washing the print in order to eliminate the fixing reagent.

The foregoing specification of our improved process of photography in colors is signed by us this ninth day of March 1910.

AUGUSTE JEAN BAPTISTE TAULEIGNE.

ELIE MAZO.

Witnesses:

H. C. COKE,

R. THIRIOT.